

1

2,892,705

STABLE, HIGH STRENGTH, ALPHA TITANIUM  
BASE ALLOYS

Robert I. Jaffee, Worthington, and Horace R. Ogden, Columbus, Ohio, and Milton B. Vordahl, Beaver, Pa., assignors, by mesne assignments, to Crucible Steel Company of America, Flemington, N.J., a corporation of New Jersey

No Drawing. Application March 8, 1957  
Serial No. 644,713

14 Claims. (Cl. 75—175.5)

This invention pertains to strong, ductile and thermally stable, alpha alloys of titanium, which are characterized by high strength and ductility at both room and elevated temperatures, and which retain these properties on prolonged exposure to elevated temperatures in both stressed and unstressed conditions.

We have previously shown in Patents 2,669,513; 2,669,514; 2,703,278; and 2,779,677, that alpha titanium alloys containing aluminum, tin and antimony singly and in combination, have excellent strength and ductility properties over the ranges of about 0.5-8% aluminum, 1-23% tin and 1-18% antimony.

Our original investigations indicated that the aforesaid alloys containing any one or more of aluminum, tin and antimony within the ranges aforesaid, were all single phase, alpha alloys. We have now discovered that under certain conditions, an ordered or partially ordered arrangement of the titanium and alloy atoms is obtained in alloys containing one or more of these elements aluminum, tin and antimony in amounts above a certain critical upper limit. Our investigations indicate that this ordered structure results from the formation of a  $Ti_3Al$  phase, a  $Ti_3Sn$  phase, a  $Ti_3Sb$  phase, or if more than one alpha stabilizer of this group is present, the aluminum, tin and antimony combine to form a  $Ti_2Al$ ,  $Ti_2Sn$ ,  $Ti_2Sb$  phase. That is to say, when any two or more of aluminum, tin and antimony are present in the alloy, the atoms of these elements will appear indiscriminately and in random sequence in the ordering, without affecting the building up of the ordered structure. The composition of the completely ordered structure thus corresponds to  $Ti_3Al$ ,  $Ti_3Sn$ ,  $Ti_3Sb$ , if these elements are present individually, or to  $Ti_3(Al, Sn, Sb)$  if any two or more are present, and occurs at about 25 atomic percent of these alloying additions, or at about 16, 45 and 46 weight percent, for Al, Sn and Sb, respectively.

The conditions under which this ordered phase starts to form are prolonged exposure at elevated temperatures of about 800-1000° F. Strain caused by stress appears to accelerate the formation of this ordering, particularly where the material is stressed at elevated temperatures on the order of 800-1000° F.

For titanium-aluminum binary alloys, our investigations have shown that this ordering becomes sufficiently pronounced markedly to decrease ductility during aging, at around 6 to 8% by weight of aluminum, i.e., at about 6-7% aluminum if the aging is conducted at around 800° F. and at about 7-8% aluminum if the aging is effected at about 1000° F. In the case of titanium-tin and titanium-antimony binary alloys, the ordering tendency becomes pronounced at about 22-27 weight percent of the tin and/or antimony.

Our investigations have further shown that insofar as concerns their effects on this tendency toward ordering, about 3% by weight of tin or antimony is equivalent to about 1% by weight of aluminum. Thus, where two or all of these elements are present, the equivalent alumini-

2

num content for purposes of computing the ordering tendency is equal to the sum of the aluminum content plus  $\frac{1}{3}$  times the tin content plus  $\frac{1}{3}$  times the antimony content, considered on a weight percent basis.

5 Thus the ordering tendency will become pronounced if the equivalent aluminum content of the alloy, computed in this manner, is upwards of about 7%, where any one, two or all of the elements aluminum, tin and antimony are present in the alloy. Or expressed more exactly in terms of atomic percent, the ordering becomes pronounced at 800° F. if the total atomic percent of the aluminum, tin and antimony present in the alloy is upwards of about 10.5 atomic percent and at 1000° F. if the total atomic percent of these elements is upwards of about 12.5 atomic percent.

10 The formation of this ordered structure causes a loss in ductility of these alloys. Although the alpha alloys of the above patents have, in the condition as annealed above the maximum temperature at which ordering occurs or as 15 quenched to room temperature therefrom, excellent strength and ductility at room temperature, nevertheless if these alloys containing above the critical aluminum equivalent content aforesaid, are subjected to prolonged service at temperatures around 800-1000° F., loss in 20 ductility will occur. And since the strength of these alloys is dependent on the total alloy content, the maximum strength of these  $Ti-(Al, Sn, Sb)$  alloys, suitable for use at temperatures of 800-1000° F. will be limited by the maximum or critical equivalent aluminum content 25 aforesaid.

30 Now we have discovered, in accordance with one aspect of our present invention, that zirconium additions to alpha alloys containing one or more of aluminum, tin and antimony, will produce strengthening of these alloys without 35 promoting the formation of the ordered  $Ti_3(Al, Sn, Sb)$  type of phase, so long as the equivalent aluminum content is less than 6% by weight or less than 10.5 atomic percent of the alloy. Therefore, the maximum strength obtainable in a stable alpha alloy of this type will be greater for 40 alloys containing zirconium than for those in which no zirconium is present. The zirconium added to such alpha alloys replaces part of the titanium in the  $Ti_3(Al, Sn, Sb)$  compound, which can thus be expressed as  $(Ti, Zr)_3(Al, Sn, Sb)$ , and does not alter significantly the critical equivalent 45 aluminum content of 7 weight percent at which ordering becomes pronounced. Thus, for example, we have found that a Ti-4Al-12Sn alloy, the equivalent aluminum content of which as above computed, is 8.0% by weight, is unstable; while a Ti-4Al-12Zr alloy having an equivalent aluminum content of 4% by weight is stable; and also that a Ti-6Al-6Zr alloy having an equivalent aluminum content of 6% by weight is stable.

50 In our discussion thus far, we have confined attention to the alpha promoters aluminum, tin and antimony which enter the ordered position X in the ordered phase  $Ti_3X$ , and to zirconium, which substitutes, as noted above, for part of the titanium in the ordered phase and hence does not promote ordering. Additional alpha promoters which 55 enter the ordered position X when they dissolve in alpha titanium are silver and indium, which thus up to the limits of their solubilities in alpha titanium, are susceptible to the formation of ordered phases of the type  $Ti_3Ag$ , and  $Ti_3In$ . Indium is soluble in alpha titanium up to about 3% by weight, and silver up to about 10% by weight. Within these limits of alpha solubility, additions 60 of these elements will therefore increase the strength of alpha titanium alloys, but if ordering embrittlement is to be avoided, silver and indium like aluminum, tin and antimony, must not be present in the alloy in total amount 65 of more than about 10.5 atomic percent.

Additional elements which, like zirconium, do not enter the ordered position X in the  $Ti_3X$  lattice, and therefore do not contribute to ordering, but which at the same time, produce strengthening of alpha titanium alloys, up to the limits of their alpha solubilities therein, are hafnium, and the various beta promoters such as vanadium, columbium, tantalum, molybdenum, manganese, iron, chromium, tungsten, cobalt, etc. Only a few of these beta promoters, however, have sufficient solubility in alpha titanium to impart material strengthening to alpha titanium alloys. They are tantalum which is alpha soluble up to about 10% by weight, columbium and vanadium which are alpha soluble up to about 3% by weight, and molybdenum and manganese which are alpha soluble up to about 0.5% by weight of each. The alpha solubilities of beta promoters like chromium, tungsten, iron, cobalt, nickel, copper and silicon are so low as not to permit of significant amounts of strengthening of alpha titanium alloys, but to the extent that these elements are soluble in alpha titanium, they will act like zirconium in that they will permit equivalent strengthening by substituting for part of the titanium and will not take up ordered positions in the lattice.

Since zirconium and hafnium are isomorphous with titanium, and produce only alpha alloys therewith at room or atmospheric temperature, they may accordingly be substituted for titanium in all proportions. A preferred range for zirconium as an alpha strengthener is, however, about 4 to 15%.

Thus to summarize, the general formula for the completely ordered structure with reference to those of the elements above mentioned which have appreciable solubilities in alpha titanium is as follows:

(Ti, Zr, Hf, V, Cb, Ta, Mo, Mn)<sub>3</sub>(Al, Sn, Sb, Ag, In)

All elements in the above formula must, as stated, be present only within the limits of alpha solubility for each or in total amount in the production of a high strength, alpha alloys of titanium. Furthermore, if ordering embrittlement of the alloy due to aging at 800-1000° F. is to be avoided, the total content of the elements which take up ordered positions in the  $Ti_3X$  lattice, namely, those which substitute for X therein, shall not exceed 10.5 atomic percent of the total alloy content, these being, as above stated, the elements aluminum, tin, antimony, silver and indium.

Since the atomic weights of tin, antimony, silver and

indium are close to one another, falling within the range of about 115-122 in round numbers, they will have approximately the same effect on the ordering tendency when alloyed with titanium, on an equal weight percent basis, i.e., percent-for-percent of each. And since as shown above, the equivalent aluminum content of tin and antimony on a weight percent basis is approximately  $\frac{1}{3}$  times the weight percent of each present in the alloy, the same rule applies for silver and indium. Thus the general formula for the equivalent aluminum content on a weight percent basis is the sum of the aluminum content plus  $\frac{1}{3}$  times the total weight percent of tin, antimony, silver and indium present in the alloy. If the equivalent aluminum as thus computed is under 6%, the alloy is stable, and if over 7% the alloy is unstable. The critical limit of 6 weight percent of equivalent aluminum corresponds to the critical limit of 10.5 atomic percent of these elements present.

Since the alloying additions are usually given in terms of weight percent of each, the conversion to atomic percent for determining the ordering tendency is computed from the fraction in which the sum of the weight percent divided by the atomic weight of each of Al, Sn, Sb, Ag and In, appears in the numerator, while the sum of the weight percent divided by the atomic weight of each and every element present in the alloy appears in the denominator. If the fraction as thus computed is under 0.105, i.e., under 10.5 percent, the alloy is stable and if above this amount, the alloy is unstable.

As illustrative of the invention as thus described, reference will now be had to the test results in the following Table I, based on a series of alloy ingots produced by arc melting titanium sponge of commercial purity except as otherwise indicated, together with the alloying ingredients, in a cold mold furnace, in an inert atmosphere. The ingots were forged into plate at about 2000° F., and rolled into sheet or bar stock at about 1600° F. finishing temperature, were then annealed 7 hours at 1600° F. and air cooled to room temperature. As shown by the data in the table, bar or sheet specimens, as indicated, of each of the alloys as thus produced, were tested for room temperature tensile properties in the "as annealed" condition, and also after aging exposure for at least 100 hours at 800° F. and 1000° F., in unstressed and/or stressed condition as shown. The alloys were also tensile tested at 1000° F., with results as shown in the table.

TABLE I

| Composition, Percent (Balance Titanium) | Specimen Type | Time, Hrs. | Temp., F. | Stress, 1,000 p.s.i. | Per- cent Plastic Strain | Min. Creep Rate per hr. | Test Temp., F. | Tensile Prop- erties, p.s.i. $\times$ 1,000 |           | Percent Elonga- tion in 1" | Percent Reduc- tion in Area | MBR, T |   |
|-----------------------------------------|---------------|------------|-----------|----------------------|--------------------------|-------------------------|----------------|---------------------------------------------|-----------|----------------------------|-----------------------------|--------|---|
|                                         |               |            |           |                      |                          |                         |                | 0.2% Offset Yield                           | Ult. Str. |                            |                             | L      | T |
| 6Al-6Sn, RES-1435-15 (iodide base).     | Bar (T)...    | None       |           |                      |                          |                         | 75             | 103                                         | 113       | 22                         | 47                          |        |   |
|                                         |               | 118        | 800       | None                 |                          |                         | 75             | 113                                         | 114       | 20                         | 48                          |        |   |
|                                         |               | 138        | 800       | 65                   | 4.82                     | 0.0004                  | 75             | 117                                         | 119       | 8                          | 20                          |        |   |
|                                         | Bar (T)...    | 120        | 1,000     | None                 |                          |                         | 75             | 114                                         | 114       | 8                          | 17                          |        |   |
|                                         |               | None       |           |                      |                          |                         | 1,000          | 58                                          | 66        | 30                         | 35                          |        |   |
|                                         |               | None       |           |                      |                          |                         | 75             | 116                                         | 119       | 10                         | 13                          |        |   |
| 6Al-6Sn, RES-1435-16 (sponge base).     | Bar (T)...    | 118        | 800       | None                 |                          |                         | 75             | 113                                         | 123       | 10                         | 14                          |        |   |
|                                         |               | 138        | 800       | 65                   | 1.34                     | 0.0005                  | 75             | 120                                         | 121       | 4                          | 12                          |        |   |
|                                         |               | 120        | 1,000     | None                 |                          |                         | 75             | 118                                         | 120       | 2                          | 8                           |        |   |
|                                         | Bar (T)...    | None       |           |                      |                          |                         | 1,000          | 62                                          | 72        | 36                         | 36                          |        |   |
|                                         |               | None       |           |                      |                          |                         | 75             | 128                                         | 129       | 4                          | 3                           |        |   |
|                                         |               | None       |           |                      |                          |                         | 75             | 128                                         | 129       | 4                          | 3                           |        |   |
| 6Al-6Sn-0.15 Ox, RES-1435-17.           | Bar (T)...    | 118        | 800       | None                 |                          |                         | 75             | 126                                         | 126       | 4                          | 7                           |        |   |
|                                         |               | 120        | 800       | 65                   | 0.09                     | Nil                     | 75             | 83                                          | 83        | 0                          | 3                           |        |   |
|                                         |               | 120        | 1,000     | None                 |                          |                         | 75             | 125                                         | 125       | 0                          | 0                           |        |   |
|                                         | (Bar (L)...   | None       |           |                      |                          |                         | 1,000          | 66                                          | 79        | 32                         | 48                          |        |   |
|                                         |               | None       |           |                      |                          |                         | 75             | 124                                         | 124       | 1                          | 3                           |        |   |
|                                         |               | None       |           |                      |                          |                         | 75             | 125                                         | 125       | 1                          | 3                           |        |   |
| 6Al-6Sn-0.3Ox, RIN-1016 R2a.            | Bar (T)...    | Bar (L)    |           |                      |                          |                         | 75             | 119                                         | 119       | 2                          | 1                           |        |   |
|                                         |               | Bar (T)    |           |                      |                          |                         | 75             | 89                                          | 89        | 2                          | 1                           |        |   |
|                                         |               | Bar (L)    |           |                      |                          |                         | 75             | 87                                          | 87        | 1                          | 0                           |        |   |
|                                         | Bar (L)...    | Bar (T)    |           |                      |                          |                         | 75             | 75                                          | 75        | 1                          | 0                           |        |   |
|                                         |               | Bar (L)    |           |                      |                          |                         | 75             | 89                                          | 89        | 0                          | 2                           |        |   |
|                                         |               | Bar (T)    |           |                      |                          |                         | 75             | 60                                          | 60        | 0                          | 0                           |        |   |
| 6Al-6Sn-0.075N, RES-1435-18.            | Bar (T)...    | (None)     |           |                      |                          |                         | 75             | 139                                         | 139       | 2                          | 6                           |        |   |
|                                         |               | 118        | 800       | None                 |                          |                         | 75             | 139                                         | 139       | 4                          | 6                           |        |   |
|                                         |               | 120        | 800       | 65                   | 0.34                     | 0.0004                  | 75             | 106                                         | 106       | 0                          | 3                           |        |   |
|                                         | Bar (T)...    | 1,000      |           | None                 |                          |                         | 75             | 95                                          | 95        | 0                          | 3                           |        |   |
|                                         |               | 120        | 1,000     | None                 |                          |                         | 75             | 61                                          | 73        | 24                         | 39                          |        |   |
|                                         |               | None       |           |                      |                          |                         | 1,000          | 61                                          | 73        | 24                         | 39                          |        |   |

TABLE I—Continued

| Composition, Percent (Balance Titanium) | Specimen Type | Time, Hrs. | Temp., F. | Stress, 1,000 p.s.i. | Per- cent Plastic Strain | Min. Creep Rate per hr. | Test Temp., F. | Tensile Prop- erties, p.s.i. $\times$ 1,000 |           | Percent Elonga- tion in 1" | Percent Reduction in Area | MBR, T |     |
|-----------------------------------------|---------------|------------|-----------|----------------------|--------------------------|-------------------------|----------------|---------------------------------------------|-----------|----------------------------|---------------------------|--------|-----|
|                                         |               |            |           |                      |                          |                         |                | 0.2% Offset Yield                           | Ult. Str. |                            |                           | L      | T   |
| 6Al-6Sn-0.075C, RES-1435-19.            | Bar (T)       | None       |           |                      |                          |                         | 75             | 129                                         | 131       | 12                         | 12                        |        |     |
|                                         |               | 118        | 800       | None                 |                          |                         | 75             | 127                                         | 131       | 4                          | 8                         |        |     |
|                                         |               | 120        | 800       | 65                   | (1)                      | (1)                     | 75             | 132                                         | 132       | 6                          | 14                        |        |     |
|                                         |               | 120        | 1,000     | None                 |                          |                         | 75             | 132                                         | 132       | 0                          | 5                         |        |     |
|                                         |               | None       |           |                      |                          |                         | 1,000          | 66                                          | 76        | 42                         | 45                        |        |     |
|                                         |               | None       |           |                      |                          |                         | 75             | 129                                         | 134       | 8                          | 11                        |        |     |
|                                         |               | 118        | 700       | None                 |                          |                         | 75             | 133                                         | 133       | 4                          | 6                         |        |     |
|                                         |               | 120        | 800       | 65                   | (1)                      | (1)                     | 75             | 135                                         | 136       | 2                          | 9                         |        |     |
|                                         |               | 120        | 1,000     | None                 |                          |                         | 75             | 135                                         | 136       | 3                          | 6                         |        |     |
|                                         |               | None       |           |                      |                          |                         | 1,000          | 73                                          | 89        | 20                         | 40                        |        |     |
| 6Al-6Sn-0.5Fe, RES-1435-20.             | Bar (T)       | None       |           |                      |                          |                         | 75             | 134                                         | 145       | 15                         | 31                        |        |     |
|                                         |               | None       |           |                      |                          |                         | 75             | 129                                         | 140       | 4                          | 8                         |        |     |
|                                         |               | 118        | 700       | None                 |                          |                         | 75             | 140                                         | 147       | 8                          | 15                        |        |     |
|                                         |               | 120        | 800       | 65                   | (1)                      | (1)                     | 75             | 135                                         | 136       | 12                         | 59                        |        |     |
|                                         |               | 120        | 1,000     | None                 |                          |                         | 75             | 129                                         | 134       | 14                         | 39                        |        |     |
|                                         |               | None       |           |                      |                          |                         | 75             | 125                                         | 130       | 11                         | 44                        |        |     |
|                                         |               | None       |           |                      |                          |                         | 75             | 129                                         | 130       | 2                          | 9                         |        |     |
|                                         |               | 97         | 800       | 65                   | 0.128                    | 0.0013                  | 75             | 135                                         | 135       | 6                          | 7                         |        |     |
|                                         |               | 97         | 1,000     | 15                   | 0.145                    | 0.0009                  | 75             | 129                                         | 134       | 18                         | 35                        |        |     |
|                                         |               | None       |           |                      |                          |                         | 1,000          | 79                                          | 88        | 30                         | 31                        |        |     |
| 6Al-6Sn-1Mo, RES-1435-29.               | Bar (T)       | None       |           |                      |                          |                         | 75             | 129                                         | 134       | 14                         | 15                        |        |     |
|                                         |               | None       |           |                      |                          |                         | 75             | 125                                         | 130       | 8                          | 17                        |        |     |
|                                         |               | 96         | 800       | 65                   | 0.128                    | 0.0013                  | 75             | 129                                         | 140       | 4                          | 8                         |        |     |
|                                         |               | 97         | 1,000     | 15                   | 0.145                    | 0.0009                  | 75             | 140                                         | 147       | 8                          | 15                        |        |     |
|                                         |               | None       |           |                      |                          |                         | 1,000          | 79                                          | 88        | 12                         | 59                        |        |     |
|                                         |               | None       |           |                      |                          |                         | 75             | 125                                         | 130       | 11                         | 44                        |        |     |
|                                         |               | None       |           |                      |                          |                         | 75             | 129                                         | 134       | 14                         | 39                        |        |     |
|                                         |               | 97         | 800       | 65                   | 0.106                    | 0.0011                  | 75             | 135                                         | 135       | 2                          | 9                         |        |     |
|                                         |               | 100        | 1,000     | 15                   | 0.005                    | 0.0005                  | 75             | 129                                         | 134       | 18                         | 35                        |        |     |
|                                         |               | None       |           |                      |                          |                         | 1,000          | 70                                          | 80        | 30                         | 31                        |        |     |
| 6Al-6Sn-2V, RES-1435-30.                | Bar (T)       | None       |           |                      |                          |                         | 75             | 114                                         | 117       | 12                         | 24                        |        |     |
|                                         |               | None       |           |                      |                          |                         | 75             | 121                                         | 121       | 12                         | 24                        |        |     |
|                                         |               | 95         | 800       | 65                   | 0.375                    | 0.0004                  | 75             | 120                                         | 121       | 8                          | 17                        |        |     |
|                                         |               | 113        | 1,000     | 15                   | 0.010                    | 0.0004                  | 75             | 110                                         | 113       | 2                          | 6                         |        |     |
|                                         |               | None       |           |                      |                          |                         | 75             | 131                                         | 131       | 2                          | 6                         |        |     |
|                                         |               | None       |           |                      |                          |                         | 75             | 130                                         | 132       | 2                          | 12                        |        |     |
|                                         |               | 118        | 800       | 65                   | (1)                      | (1)                     | 75             | 126                                         | 133       | 1                          | 2                         |        |     |
|                                         |               | 120        | 800       | 65                   | (1)                      | (1)                     | 75             | 124                                         | 129       | 20                         | 38                        | 3.1    | 3.0 |
|                                         |               | 120        | 1,000     | None                 |                          |                         | 75             | 126                                         | 133       | 12                         | 40                        |        |     |
|                                         |               | None       |           |                      |                          |                         | 1,000          | 66                                          | 84        | 22                         | 48                        |        |     |
| 6Al-6Sn-3Cb, RES-1435-31.               | Bar (T)       | None       |           |                      |                          |                         | 75             | 114                                         | 120       | 28                         | 36                        | 6.7    | 9.0 |
|                                         |               | 95         | 800       | 65                   | 0.375                    | 0.0004                  | 75             | 116                                         | 119       | 12                         | 13                        |        |     |
|                                         |               | 113        | 1,000     | 15                   | 0.010                    | 0.0004                  | 75             | 117                                         | 120       | 18                         | 24                        |        |     |
|                                         |               | None       |           |                      |                          |                         | 75             | 131                                         | 131       | 2                          | 6                         |        |     |
|                                         |               | None       |           |                      |                          |                         | 75             | 130                                         | 132       | 2                          | 12                        |        |     |
|                                         |               | 118        | 800       | 65                   | (1)                      | (1)                     | 75             | 126                                         | 133       | 1                          | 2                         |        |     |
|                                         |               | 120        | 800       | 65                   | (1)                      | (1)                     | 75             | 124                                         | 129       | 20                         | 38                        | 3.1    | 3.0 |
|                                         |               | 120        | 1,000     | None                 |                          |                         | 75             | 126                                         | 133       | 12                         | 40                        |        |     |
|                                         |               | None       |           |                      |                          |                         | 1,000          | 66                                          | 84        | 22                         | 48                        |        |     |
|                                         |               | None       |           |                      |                          |                         | 75             | 114                                         | 120       | 28                         | 36                        | 6.7    | 9.0 |
| 4Al-12Zr, RES-1435-24.                  | Bar (T)       | 98         | 800       | 65                   | 0.624                    | 0.0021                  | 75             | 116                                         | 119       | 12                         | 13                        |        |     |
|                                         |               | 114        | 800       | 65                   | 0.741                    | b 0.0009                | 75             | 117                                         | 120       | 18                         | 24                        |        |     |
|                                         |               | 96         | 1,000     | 15                   | 0.150                    | 0.0011                  | 75             | 116                                         | 119       | 18                         | 35                        |        |     |
|                                         |               | 97         | 1,000     | 15                   | 0.175                    | b 0.0014                | 75             | 116                                         | 118       | 22                         | 37                        |        |     |
|                                         |               | None       |           |                      |                          |                         | 75             | 118                                         | 122       | 15                         | 31                        | 3.9    | 2.7 |
|                                         |               | None       |           |                      |                          |                         | 75             | 122                                         | 123       | 8                          | 18                        |        |     |
|                                         |               | 100        | 800       | 65                   | 0.190                    | NiI                     | 75             | 122                                         | 125       | 4                          | 9                         |        |     |
|                                         |               | 100        | 800       | 65                   | 0.399                    | b NiI                   | 75             | 125                                         | 125       | 22                         | 39                        |        |     |
|                                         |               | 97         | 1,000     | 15                   | 0.010                    | b 0.001                 | 75             | 124                                         | 124       | 12                         | 39                        |        |     |
|                                         |               | None       |           |                      |                          |                         | 1,000          | 64                                          | 78        | 25                         | 49                        |        |     |
| 5Al-5Sn-5Zr, RES-1435-25.               | Bar (T)       | None       |           |                      |                          |                         | 75             | 128                                         | 136       | 29                         | 43                        | 3.3    | 2.5 |
|                                         |               | None       |           |                      |                          |                         | 75             | 128                                         | 129       | 2                          | 8                         |        |     |
|                                         |               | 100        | 800       | 65                   | 0.306                    | 0.0009                  | 75             | 128                                         | 137       | 23                         | 31                        |        |     |
|                                         |               | 100        | 800       | 65                   | 1.010                    | b 0.0008                | 75             | 137                                         | 140       | 18                         | 31                        |        |     |
|                                         |               | 96         | 800       | 65                   | 0.065                    | b 0.0008                | 75             | 133                                         | 140       | 26                         | 40                        |        |     |
|                                         |               | 98         | 1,000     | 15                   | 0.065                    | b 0.0001                | 1,000          | 76                                          | 93        | 18                         | 20                        | 3.6    | 2.0 |
|                                         |               | None       |           |                      |                          |                         | 75             | 128                                         | 130       | 30                         | 32                        |        |     |
|                                         |               | 118        | 800       | 65                   | 0.140                    | 0.0008                  | 75             | 126                                         | 132       | 3                          | 9                         |        |     |
|                                         |               | 95         | 800       | 65                   | 0.086                    | b NiI                   | 75             | 132                                         | 132       | 8                          | 10                        |        |     |
|                                         |               | 95         | 800       | 65                   | 0.025                    | b 0.0001                | 75             | 132                                         | 133       | 4                          | 5                         |        |     |
| 6Al-6Sn-6Zr, RES-1435-27.               | Bar (T)       | None       |           |                      |                          |                         | 1,000          | 79                                          | 89        | 30                         | 32                        |        |     |
|                                         |               | None       |           |                      |                          |                         | 75             | 113                                         | 115       | 23                         | 33                        | 2.6    | 2.6 |
|                                         |               | 100        | 800       | 65                   | 4.420                    | 0.0006                  | 75             | 113                                         | 113       | 11                         | 26                        |        |     |
|                                         |               | 112        | 800       | 65                   | 10.000                   | b NiI                   | 75             | 104                                         | 104       | 16                         | 47                        |        |     |
|                                         |               | 99         | 1,000     | 15                   | 0.028                    | b 0.005                 | 75             | 117                                         | 118       | 14                         | 31                        |        |     |
|                                         |               | None       |           |                      |                          |                         | 1,000          | 55                                          | 67        | 30                         | 35                        |        |     |
|                                         |               | None       |           |                      |                          |                         | 75             | 134                                         | 145       | 15                         | 31                        | 2.3    | 3.5 |
|                                         |               | None       |           |                      |                          |                         | 75             | 129                                         | 140       | 4                          | 8                         |        |     |
|                                         |               | 96         | 800       | 65                   | 0.128                    | 0.0013                  | 75             | 129                                         | 140       | 2                          | 20                        |        |     |
|                                         |               | 111        | 800       | 65                   | 0.255                    | b 0.0010                | 75             | 127                                         | 140       | 12                         | 20                        |        |     |
| 6Al-6Sn-2V, RES-1435-30.                | Bar (T)       | None       |           |                      |                          |                         | 75             | 140                                         | 147       | 8                          | 15                        |        |     |
|                                         |               | 97         | 800       | 65                   | 0.106                    | 0.0011                  | 75             | 127                                         | 130       | 2                          | 7                         |        |     |
|                                         |               | 100        | 1,000     | 15                   | 0.005                    | b 0.0005                | 75             | 135                                         | 135       | 6                          | 7                         |        |     |
|                                         |               | None       |           |                      |                          |                         | 1,000          | 70                                          | 80        | 18                         | 35                        |        |     |
|                                         |               | None       |           |                      |                          |                         | 75             | 114                                         | 117       | 30                         | 31                        | 2.6    | 3.3 |
|                                         |               | 97         | 800       | 65                   | 0.375                    | 0.0004                  | 75             | 121                                         | 121       | 14                         | 15                        |        |     |
|                                         |               | 97         | 800       | 65                   | 0.300                    | b 0.0006                | 75             | 116                                         | 118       | 10                         | 24                        |        |     |
|                                         |               | 113        | 1,000     | 15                   | 0.010                    | b 0.0003                | 75             | 120                                         | 121       | 8                          | 17                        |        |     |
|                                         |               | None       |           |                      |                          |                         | 1,000          | 61                                          | 67        | 15                         | 38                        |        |     |
|                                         |               | None       |           |                      |                          |                         | 75             | 140                                         | 148       | 20                         | 51                        |        |     |
| 6Al-6Sn-3Cb, RES-1435-31.               | Bar (T)       | 71         | 800       | 50                   | 0.36                     | 0.004                   | 75             | 147                                         | 158       | 20                         | 37                        |        |     |
|                                         |               | 112        | 1,000     | 15                   | 1.54                     | 0.012                   | 75             | 132                                         | 142       | 15                         | 36                        |        |     |
|                                         |               | None       |           |                      |                          |                         | 75             | 134                                         | 142       | 14                         | 20                        |        |     |
|                                         |               | 104        | 800       | 60                   | 0.06                     | b 0.0003                | 75             | 137                                         | 146       | 7                          | 15                        |        |     |
|                                         |               | 98         | 800       | 65                   | 0.09                     | 0.0006                  | 75             | 137                                         | 145       | 10                         | 18                        |        |     |
|                                         |               | 104        | 1,000     | 10                   | 0.10                     | b 0.0005                | 75             | 135                                         | 143       | 9                          | 18                        |        |     |
|                                         |               | 99         | 1,000     | 15                   | 0.19                     | b 0.0012                | 75             | 134                                         | 141       | 12                         | 20                        |        |     |
|                                         |               | None       |           |                      |                          |                         | 75             | 150                                         | 157       | 12                         | 21                        |        |     |
|                                         |               | 97         | 800       | 65                   | 0.079                    | b NiI                   | 75             | 151                                         | 162       | 7                          | 9                         |        |     |
|                                         |               | 98         | 1,000     | 25                   | 0.436                    | b 0.0038                | 75             | 150                                         | 159       | 12                         | 10                        |        |     |
| 4Al-12Zr-3Cu, RES-1435-41-47, inc.      | Bar (T)       | 69         | 1,000     | 15                   | 0.056                    | b 0.0016                | 75             | 146                                         | 156       | 10                         | 23                        |        |     |
|                                         |               | 99         | 800       | 75                   | 0.105                    | b 0.0060                | 75             |                                             |           |                            |                           |        |     |

As shown by the test results in the foregoing table, it will be seen that all analyses having equivalent aluminum of 6 or under on a weight percent basis, showed excellent stability after creep exposure for approximately 100 hours at 800° F. and 65,000 p.s.i., and at 1000° F. and 15,000 p.s.i. stress, such, for example, as the Ti-5Al-2.5Sn, Ti-4Al-12Zr, Ti-6Al-6Zr and Ti-4Al-4Sn-10Zr analyses. In contrast, all of the analyses containing equivalent aluminum of more than 6 showed instability in varying degrees as a result of such aging and creep exposure tests, such for example, as the Ti-6Al-6Sn analyses with and without other additions, as indicated, and the Ti-5Al-5Sn-5Zr, Ti-5Al-5Sn-10Zr and Ti-4Al-6Sn-6Sb analyses.

Referring to the stable alloys of the first group, the 15 Ti-5Al-2.5Sn alloy retained excellent ductility of 15-20% tensile elongation before and after all exposure tests, combined with a high tensile strength of 140,000-160,000 p.s.i. The same is true of the Ti-4Al-12Zr and Ti-6Al-6Zr alloys which maintained tensile elongations of 12-22% and 11-16% after exposure. Similarly, the Ti-4Al-4Sn-10Zr alloy maintained excellent tensile elongation of 12-24% before and after creep exposure with an ultimate strength of about 130,000 p.s.i.

The copper-bearing analyses containing equivalent aluminum under 6 were not quite so stable as those above discussed, because copper reacts with the titanium to form the compound  $Ti_2Cu$ , which thus increases the percentage of aluminum or its equivalent present in the remaining alpha matrix, and which also tends to precipitate out during aging exposure and thus tends to reduce ductility. Copper, however, has a marked strengthening action on the alloy as shown by the ultimate strengths varying from about 140,000 to 160,000 p.s.i. for the Ti-12Zr-3Cu and the Ti-6Al-6Zr-3Cu alloys. These alloys also having excellent creep strength as shown in the table. Likewise, the Ti-5Al-12Zr-6Cu alloy in addition to extremely high strength of about 160,000 p.s.i. has quite good stability, with tensile elongations maintained being about 10-12% before and after creep exposure.

All rapidly eutectoid compound-forming elements, such as cobalt, nickel, silicon, beryllium, etc., have the same effect as copper, in that they react with and tie up some of the titanium, thereby to increase the atomic percentage of aluminum and equivalent atoms present in the alpha matrix.

The effect of the various interstitial and beta promoter additions within the limits of alpha-solubility, as shown in the table, is somewhat masked by the fact that these additions were made in each instance to the Ti-6Al-6Sn base alloy containing equivalent aluminum of 8% and hence above the limit of 6 for stability, the base alloy itself being unstable for this reason as shown by the Ti-6Al-6Sn analyses containing no such additions. It will be seen, however, by comparison that alpha soluble

columbium additions, improve ductility of this base alloy on aging. Thus such columbium additions improve stability even for these alloys containing up to 7 or 8% by weight of equivalent aluminum.

Alpha soluble vanadium additions have the same stabilizing action. Thus a Ti-12Sn-4Al alloy containing the 8% aluminum equivalent had in the as quenched condition from 1500° F., a tensile elongation of 4% and an area reduction of 3%, which values were reduced to zero on aging for 100 hours at 1000° F. In contrast, a Ti-12Sn-4Al-2V alloy had as quenched from 1500° F., a tensile elongation of 10% and an area reduction of 18%. On aging for 200 hours at 1000° F., the tensile elongation was found to be 10% and the area reduction 22%. Thus the alpha soluble addition of 2% vanadium to the Ti-12Sn-4Al base alloy transformed it from a highly unstable to a highly stable alloy. Other tests have shown that alpha soluble molybdenum and tantalum additions impart a similar stabilizing action.

As to the interstitial additions, carbon, oxygen and nitrogen, it will be seen from Table I that they have a generally detrimental effect on stability, and hence are not desirable additions to alpha alloys as adjudged from this standpoint, despite the increase in strength imparted thereby.

The alloys of the invention have good welding properties as shown by the test results in the following Table II:

TABLE II  
Bend-test results for alpha alloys before and after welding  
[Annealed 4 hours at 1600° F. and air cooled.]

| Alloy No.   | Composition, percent<br>(Balance Titanium) | Minimum Bend<br>Radius, T, Longi-<br>tudinal |        |
|-------------|--------------------------------------------|----------------------------------------------|--------|
|             |                                            | Base                                         | Welded |
| RES-1435-23 | 4Al-4Sn-10Zr                               | 3.1                                          | 7.2    |
| PA-2212     | 4Al-4Sn-10Zr                               | 5.2                                          | 5.3    |
| RES-1435-24 | 4Al-12Zr                                   | 6.7                                          | 4.0    |
| PA-2213     | 4Al-12Zr                                   | 3.5                                          | 6.8    |
| RES-1435-25 | 5Al-5Sn-5Zr                                | 3.9                                          | 4.0    |
| PA-2214     | 5Al-5Sn-5Zr                                | 2.5                                          | 7.4    |
| RES-1435-26 | 5Al-5Sn-10Zr                               | 3.3                                          | 5.8    |
| PA-2215     | 5Al-5Sn-10Zr                               | 4.6                                          | 8.0    |
| RES-435-27  | 6Al-6Sn-6Zr                                | 3.6                                          | 5.3    |
| PA-2216     | 6Al-6Sn-6Zr                                | 4.4                                          | 7.6    |
| RES-1435-28 | 6Al-6Zr                                    | 2.6                                          | 2.3    |
| PA-2217     | 6Al-6Zr                                    | 2.6                                          | 3.7    |
| RES-1435-29 | 6Al-6Sn-1Mo                                | 2.3                                          | 6.7    |
| RES-1435-30 | 6Al-6Sn-2V                                 | 2.9                                          | 5.8    |
| RES-1435-31 | 6Al-6Sn-3Cb                                | 2.6                                          | 5.2    |
| PA-2210     | 6Al-3Sn-3Sb                                | 3.0                                          | 7.6    |
| PA-2211     | 4Al-6Sn-6Sb                                | 3.5                                          | 8.0    |

The room temperature mechanical properties of additional Ti-Al-Zr alloys according to the invention as annealed at 1600° F. are given in the following Table III; while the microstructures of these alloys as annealed at 1600° F. are given in the succeeding Table IV. This table also gives the 100-hour, 800° F. bend-creep and bend-creep-bend test results for this same group of alloys.

TABLE III  
Hardness, bend, and room-temperature longitudinal sheet  
tensile test results for Ti-Al-Zr alpha alloys  
[Annealed 7 hours at 1600° F. and air cooled to room temperature.]

| Alloy Number | Composition,<br>percent (Bal-<br>ance Titanium) | Tensile Properties:<br>p.s.i. $\times 1,000$ |                      | Percent<br>Elongation<br>in 1" | Percent<br>Reduction<br>in Area | VHN     | MBR, T<br>(Long.) |
|--------------|-------------------------------------------------|----------------------------------------------|----------------------|--------------------------------|---------------------------------|---------|-------------------|
|              |                                                 | 0.2% Offset<br>Yield                         | Ultimate<br>Strength |                                |                                 |         |                   |
| PA-2240      | 4Al-6Zr                                         | 89                                           | 94                   | 15                             | 37                              | 310     | 3.9               |
| PA-2241      | 4Al-12Zr                                        | 106                                          | 112                  | 13                             | 24                              | 347     | 4.0               |
| PA-2242      | 4Al-18Zr                                        | 108                                          | 114                  | 6                              | 10                              | 387     | 4.4               |
| PA-2243      | 4Al-24Zr                                        | 116                                          | 110                  | 2                              | 6                               | 374/405 | 5.7               |
| PA-2244      | 4Al-6Zr                                         | 99                                           | 105                  | 20                             | 28                              | 351     | 3.7               |
| PA-2245      | 5Al-12Zr                                        | 118                                          | 121                  | 5                              | 7                               | 365     | 4.7               |
| PA-2246      | 5Al-18Zr                                        | 127                                          | 129                  | 3                              | 6                               | 405     | 2.5/Br            |
| PA-2247      | 5Al-24Zr                                        | 132                                          | 133                  | 1                              | 5                               | 396     | Br                |
| PA-2248      | 6Al-6Zr                                         | 111                                          | 115                  | 13                             | 27                              | 386     | 3.9               |
| PA-2249      | 6Al-12Zr                                        | 122                                          | 123                  | 15                             | 35                              | 303     | 4.2               |
| PA-2250      | 6Al-18Zr                                        | 131                                          | 131                  | 9                              | 20                              | 416     | 4.2               |
| PA-2251      | 6Al-24Zr                                        | 126                                          |                      | 1                              | 3                               | 417/472 | Br                |

TABLE IV

800° F. bend-creep results and hardness and bend test results before and after bend-creep exposure on Ti-Al-Zr alloys. Structure as annealed

[Annealed 7 hours at 1600° F. and air cooled to room temperature.]

| Alloy number         | Composition, percent (Balance Titanium) | Before Exposure        |         |                | 100-Hr. 800° F. Exposure      |     |                |
|----------------------|-----------------------------------------|------------------------|---------|----------------|-------------------------------|-----|----------------|
|                      |                                         | Structure <sup>1</sup> | VHN     | MBR, T (Long.) | Residual Stress, 1,000 p.s.i. | VHN | MBR, T (Long.) |
| PA-2240              | 4Al-6Zr                                 | Trace B                | 310     | 3.9            | 33                            | 316 | 2.2            |
| PA-2241              | 4Al-12Zr                                | Trace B                | 347     | 4.0            | 46                            | 354 | 8.8            |
| PA-2242              | 4Al-18Zr                                | Approx. 5B             | 387     | 4.4            | 52                            | 358 | Br             |
| PA-2243              | 4Al-24Zr                                | Approx. 15B            | 374/405 | 5.7            | 64                            | 386 | Br             |
| PA-2244              | 5Al-6Zr                                 | Trace B                | 351     | 3.7            | 49                            | 346 | 3.8            |
| PA-2245              | 5Al-12Zr                                | Trace B                | 365     | 4.7            |                               |     |                |
| PA-2246              | 5Al-18Zr                                | Approx. 4B             | 405     | 2.5/Br         |                               |     |                |
| PA-2247              | 5Al-24Zr                                | Approx. 10B            | 396     | Br             |                               |     |                |
| PA-2248              | 6Al-6Zr                                 | Trace B                | 386     | 3.9            |                               |     |                |
| PA-2249              | 6Al-12Zr                                | Trace B                | 393     | 4.2            |                               |     |                |
| PA-2250              | 6Al-18Zr                                | Approx. 4B             | 416     | 4.2            | 64                            | 396 | Br             |
| PA-2251              | 6Al-24Zr                                | Approx. 10B            | 417/472 | Br             |                               |     |                |
| PA-2220 <sup>2</sup> | 4Al-6Zr-3Cu                             | C                      | 335     | 5.2            | 48                            | 344 | 4.9            |
| PA-2230 <sup>2</sup> | 4Al-6Zr-6Cu                             | C                      | 319     | Br             | 50                            | 332 | 9.6            |
| PA-2231 <sup>2</sup> | 4Al-12Zr-3Cu                            | C                      | 330     | 4.7            | 54                            | 341 | 4.4            |
| PA-2218 <sup>2</sup> | 4Al-12Zr-6Cu                            | C                      | 364     | Br             | 56                            | 363 | Br             |

<sup>1</sup> B=beta, C=compound. All the Ti-Al-Zr compositions are predominantly equiaxed alpha structures having the beta phase intergranularly in the described amounts. The Ti-Al-Zr-Cu compositions have both equiaxed and acicular alpha in addition to the compound phase.

<sup>2</sup> These data have been included to show the effects of a dispersoid addition on the Ti-4Al-(6, 12) Zr base. The alloys have been annealed 24 hours at 1400° F., furnace cooled to 1100° F., held 16 hrs. at 1100° F., and air cooled to room temperature.

The beta stabilizing effect of zirconium is demonstrated by the structures observed for this group of Ti-Al-Zr alpha alloys. The 1600° F. annealing temperature resulted in a two-phase structure. This varies from traces of beta phase for 6 to 12% zirconium contents, to 15% beta phase for 24% zirconium content, in a predominantly

The alloys of the invention also have good oxidation resistance at temperatures up to about 1800° F. and reasonably good oxidation resistance at about 1900° F. as shown by the test results in Table V below. The data in the lower portion of this table on unalloyed titanium and on titanium-tin and titanium-tin-aluminum alloys is added for comparison.

TABLE V  
Oxidation test data for alpha alloys

| Composition, Percent (Balance Titanium) | Weight Gain, mg./cm. <sup>2</sup> |                          |                           |                          |                          |
|-----------------------------------------|-----------------------------------|--------------------------|---------------------------|--------------------------|--------------------------|
|                                         | 24-1,560° F. <sup>a</sup>         | 4-1,600° F. <sup>b</sup> | 24-1,600° F. <sup>c</sup> | 4-1,800° F. <sup>d</sup> | 4-1,920° F. <sup>e</sup> |
| 4Al-4Sn-10Zr, RES-1435-23 <sup>f</sup>  | 6.4                               | 3.1                      | 6.0                       | 10.5                     | 64                       |
| 4Al-12Zr, RES-1435-24                   | 6.1                               | 3.1                      | 7.5                       | 9.6                      | 35                       |
| 5Al-5Sn-5Zr, RES-1435-25                | 5.3                               | 1.9                      | 5.8                       | 9.2                      | 51                       |
| 5Al-5Sn-10Zr, RES-1435-26               | 4.9                               | 3.1                      | 9.3                       | 13.9                     | 35                       |
| 6Al-6Sn-6Zr, RES-1435-27                | 4.6                               | 2.6                      | 7.5                       | 12.5                     | 53                       |
| 6Al-6Zr, RES-1435-28                    | 3.8                               | 2.4                      | 6.4                       | 10.3                     | 28                       |
| 6Al-6Sn-1Mo, RES-1435-29                | 9.0                               | 8.3                      | 24.3                      | 18.9                     | 44                       |
| 6Al-6Sn-2V, RES-1435-30                 | 15.1                              | 4.3                      | 34.5                      | 20.1                     | 34                       |
| 6Al-6Sn-3Cb, RES-1435-31                | 2.5                               | 1.8                      | 3.6                       | 3.7                      | 8                        |
| Unalloyed, A-39                         | 14.0                              |                          |                           |                          | 35                       |
| 4Al, A-42                               | 12.0                              |                          |                           |                          |                          |
| 8Al, A-43                               | 8.5                               |                          |                           |                          |                          |

<sup>a</sup> Exposed in still air for 24 hrs. at 1,560° F. and air cooled to room temperature.

<sup>b</sup> Exposed in still air for 4 hrs. at 1,600° F. and air cooled to room temperature.

<sup>c</sup> Specimens from (b) above exposed an additional 20 hrs. at 1,600° F. and air cooled to room temperature.

<sup>d</sup> Exposed in still air for 4 hrs. at 1,800° F. and air cooled to room temperature.

<sup>e</sup> Exposed in still air for 4 hrs. at 1,920° F. and furnace cooled to room temperature.

<sup>f</sup> Alloy number.

equiaxed alpha structure. The beta is located at grain corners and intergranularly.

The foregoing data of Table I also shows that elevated-temperature strength as well as the room-temperature strength of the Ti-Al-Zr alloys is increased with increasing aluminum or zirconium content. Aluminum appears to be about five or six times as potent as zirconium at room temperature on a weight percentage basis. A decrease in ductility accompanies the increase in strength. In the 800° F. bend-creep tests of Table III, the aluminum additions again appear to be about five or six times as effective as zirconium as an alpha strengthening agent. The bend-creep-bend tests indicate that the most highly alloyed compositions are embrittled during the 100-hour, 800° F. exposure.

It will be noted from the above data that the addition of about 3% columbium imparts excellent oxidation resistance up to at least 1900° F.

The results of short time aging tests on additional alloys according to the invention, containing beta promoter additions within the limits of their alpha solubilities are shown in the following Table VI. The alloys thus tested were prepared by forging at 1800° F., followed by rolling at 1500° F., to 0.08", then descaled, again rolled at 1400° F. to 0.04", held 15 minutes at 1400° F., furnace-cooled therefrom to 1100° F., held one hour thereat, air cooled thence to room temperature and descaled before testing. In the table, the room temperature mechanical or tensile properties for the alloys are given for the "as rolled and annealed condition," as prepared, supra, in

cluding minimum bend values, and the minimum bend values are also given for some of the alloys after aging for 48 hours at 750° F.

14%, iron about 8%, nickel, cobalt and copper about 5%, and silicon and beryllium about 2%.

Oxidation test data for such alpha-beta alloys in com-

TABLE VI  
Mechanical and aging properties of ternary Ti-Al-beta-isomorphous alloys

| Composition,<br>Percent<br>(Balance<br>Titanium) | Tensile Properties:<br>p.s.i. X 1,000 |                      | Percent<br>Elongation<br>in 1" | Percent<br>Reduction<br>in Area | VHN | Min. Bend Rad. T              |     |     |     |  |  |  |
|--------------------------------------------------|---------------------------------------|----------------------|--------------------------------|---------------------------------|-----|-------------------------------|-----|-----|-----|--|--|--|
|                                                  | As Rolled and<br>Annealed             |                      |                                |                                 |     | As Aged 48 Hrs.<br>at 750° F. |     |     |     |  |  |  |
|                                                  | 0.2% Off-<br>set Yield                | Ultimate<br>Strength |                                |                                 |     | L                             | T   | L   | T   |  |  |  |
| 5Al-1Cb*                                         | 89                                    | 103                  | 12                             | 40                              | 283 |                               |     |     |     |  |  |  |
| 4Al-2.5Cb                                        | 88                                    | 97                   | 20                             | 51                              | 309 | 2.3                           | 2.8 | 2.1 | 2.0 |  |  |  |
| 5Al-1Ta*                                         | 65                                    | 79                   | 19                             | 41                              | 300 |                               | 0.7 |     |     |  |  |  |
| 5Al-2.5Ta*                                       | 67                                    | 80                   | 18                             | 45                              | 276 |                               | 0.0 |     |     |  |  |  |
| 5Al-5Ta*                                         | 69                                    | 81                   | 18                             | 43                              | 294 |                               | 1.1 |     |     |  |  |  |
| 4Al-5Ta                                          | 85                                    | 93                   | 23                             | 51                              | 306 | 2.4                           | 2.4 | 1.9 | 1.9 |  |  |  |
| 4Al-10Ta                                         | 89                                    | 98                   | 20                             | 62                              | 317 | 2.4                           | 2.0 | 1.8 | 1.9 |  |  |  |
| 2.5Al-1Ag                                        | 75                                    | 86                   | 22                             | 46                              | 287 | 1.2                           | 1.6 |     |     |  |  |  |
| 2.5Al-2.5Ag                                      | 79                                    | 91                   | 22                             | 49                              | 289 | 1.5                           | 1.5 |     |     |  |  |  |
| 2.5Al-5Ag                                        | 75                                    | 89                   | 25                             | 47                              | 287 | 1.6                           | 1.5 |     |     |  |  |  |
| 2.5Al-10Ag                                       | 81                                    | 88                   | 9                              | 28                              | 317 | 1.8                           | 1.8 |     |     |  |  |  |
| 5Al-1Ag                                          | 93                                    | 102                  | 19                             | 38                              | 354 | 1.8                           | 1.8 |     |     |  |  |  |
| 5Al-2.5Ag                                        | 93                                    | 102                  | 22                             | 47                              | 342 | 1.5                           | 1.5 |     |     |  |  |  |
| 5Al-5Ag                                          | 93                                    | 106                  | 12                             | 31                              | 363 | 3.4                           | 2.7 |     |     |  |  |  |
| 5Al-1In                                          | 82                                    | 94                   | 20                             |                                 | 321 |                               | 0.7 |     |     |  |  |  |
| 5Al-2.5In                                        | 90                                    | 100                  | 17                             |                                 | 326 |                               | 1.5 |     |     |  |  |  |
| 4Al-2V                                           | 101                                   | 116                  | 12                             | 35                              | 291 | 2.4                           | 2.3 | 2.4 | 2.4 |  |  |  |
| 4Al-2.5V                                         | 96                                    | 106                  | 19                             | 51                              | 319 | 2.9                           | 5.7 | 2.5 | 2.8 |  |  |  |
| 4Al-5Ta-5Cb                                      | 121                                   | 127                  | 15                             | 44                              | 325 | 2.7                           |     | 2.7 |     |  |  |  |
| 4Al-5Ta-5V                                       | 144                                   | 145                  | 6                              | 33                              | 351 | 2.8                           |     | 3.3 |     |  |  |  |

\*Iodide base titanium; balance titanium of commercial purity.

The lower effective limit for the elements having limited solubilities in alpha titanium such as indium, vanadium, columbium, molybdenum, manganese, etc., is about 0.1%, while for those elements having higher alpha solubilities, such as zirconium, hafnium, tantalum, silver, aluminum, tin, antimony, etc., the lower effective limit is about 0.25-0.5%.

Preferred alloys according to the invention are

Ti-(3-6)Al-(4-15)Zr  
Ti-(3-6)Al-(4-10)Sn-(5-10)Zr

wherein aluminum and tin are proportioned to provide equivalent aluminum of 6 or under.

The advantages of the present invention are not confined to alloys in accordance therewith having a substantially all-alpha structure, but also apply to such as have imparted thereto a mixed alpha-beta structure due to beta promoter additions in amounts exceeding their alpha solubilities as aforesaid. The effect of such additions is simply to reduce the volume of alpha present in a given total quantity of alloy. Discrete volumes of beta are found, and in these volumes all of the beta stabilizer content beyond that soluble in the alpha is concentrated, and the amount soluble in the alpha remains as described. Hence, obviously, the stability of the remaining alpha is subject to exactly the same conditions as described for the substantially 100% alpha alloy. The most stable of such mixed phase, alpha-beta alloys are those in which the beta promoters added are isomorphous with titanium, such as molybdenum, vanadium, columbium and tantalum, with the sluggishly eutectoid beta promoters next in order such as chromium, manganese and iron, while last in order are the rapidly eutectoid beta promoters tungsten, cobalt, nickel, copper, and particularly silicon and beryllium. The mixed phase alpha-beta alloys will ordinarily not contain more than about 15-18% of such beta promoters, as beyond this they tend to have a substantially all-beta or a mixed beta-eutectoid structure at normal temperatures. For these mixed phase alpha-beta alloys, chromium and manganese should not exceed about

parison with alpha alloys according to the invention is shown in the following Table VII.

TABLE VII  
Oxidation test data for alpha and alpha-beta alloys  
[0.075-inch sheet]

| Composition, Percent<br>(Balance Titanium) | Temp.,<br>F. | Time,<br>hours | Specimen<br>Size,<br>cm. <sup>2</sup> | Weight<br>Gain,<br>mg. | Weight<br>Gain,<br>mg./cm. <sup>2</sup> |
|--------------------------------------------|--------------|----------------|---------------------------------------|------------------------|-----------------------------------------|
| 6Al-4Mo                                    | 900          | 193            | 11.7                                  | Nil                    | Nil                                     |
| 6Al-4V                                     | 900          | 193            | 13.4                                  | Nil                    | Nil                                     |
| Unalloyed                                  | 900          | 1,000          | 85.8                                  | 12.0                   | 0.14                                    |
| 5Al-2.5Sn                                  | 900          | 1,000          | 75.9                                  | 4.1                    | 0.05                                    |
| 6Al-4Mo                                    | 900          | 1,000          | 67.2                                  | 3.5                    | 0.05                                    |
| 6Al-4V                                     | 900          | 1,000          | 74.9                                  | 2.4                    | 0.03                                    |
| Unalloyed                                  | 1,000        | 1,000          | 82.0                                  | 45.7                   | 0.65                                    |
| 5Al-2.5Sn                                  | 1,000        | 1,000          | 73.2                                  | 14.5                   | 0.20                                    |
| 6Al-4Mo                                    | 1,000        | 1,000          | 69.2                                  | 14.7                   | 0.20                                    |
| 6Al-4V                                     | 1,000        | 1,000          | 68.4                                  | 24.2                   | 0.35                                    |
| 6Al-4Mo                                    | 1,100        | 193            | 9.8                                   | 5.6                    | 0.6                                     |
| 6Al-4V                                     | 1,100        | 193            | 6.9                                   | 8.2                    | 1.2                                     |
| Unalloyed                                  | 1,100        | 1,000          | 84.5                                  | 111.5                  | 1.32                                    |
| 5Al-2.5Sn                                  | 1,100        | 1,000          | 74.0                                  | 41.6                   | 0.56                                    |
| 6Al-4Mo                                    | 1,100        | 1,000          | 66.3                                  | 41.7                   | 0.63                                    |
| 6Al-4V                                     | 1,100        | 1,000          | 74.9                                  | 127.7                  | 1.73                                    |
| Unalloyed                                  | 1,200        | 1,000          | 78.9                                  | 239.8                  | 3.04                                    |
| 5Al-2.5Sn                                  | 1,200        | 1,000          | 75.6                                  | 108.3                  | 1.43                                    |
| 6Al-4Mo                                    | 1,200        | 1,000          | 68.4                                  | 94.3                   | 1.38                                    |
| 6Al-4V                                     | 1,200        | 1,000          | 68.7                                  | 361.2                  | 5.25                                    |

What is claimed is:

1. A titanium base alloy consisting essentially of about: 0.5 to 23% by weight of at least one alpha promoter selected from the group consisting of aluminum, tin, antimony, silver and indium, but not to exceed 7% of aluminum, 3% of indium and 10% of silver, and the maximum total content of the elements of said group being such that the percent of aluminum plus  $\frac{1}{3}$  times the percents of tin, antimony, silver and indium present, shall not exceed 7%, said alloy being characterized by high strength and ductility and by good stability on aging at 800-1000° C.
2. An alloy consisting essentially of about: 0.5 to 23% by weight of at least one alpha promoter selected from the group consisting of aluminum, tin, antimony,

silver and indium, but not to exceed 7% of aluminum, 3% of indium and 10% of silver, and the maximum total content of the elements of said group being such that the percent of aluminum plus  $\frac{1}{3}$  times the sum of the percents of tin, antimony, silver and indium present, shall not exceed 7%, said alloy also containing up to 50% of metal of the group zirconium and hafnium, up to 0.5% of metal of the group molybdenum and manganese, up to 3% of metal of the group columbium and vanadium, up to 10% tantalum, and the balance substantially titanium, characterized by high strength and ductility and by high thermal stability.

3. An alloy consisting essentially of about: 0.5 to 23% by weight of at least one alpha promoter selected from the group consisting of aluminum, tin, antimony, silver and indium, but not to exceed 7% of aluminum, 3% of indium and 10% of silver, and the maximum total content of the elements of said group being such that the percent of aluminum plus  $\frac{1}{3}$  times the sum of the percents of tin, antimony, silver and indium present, shall not exceed 7%, said alloy also containing about 0.25 to 50% of at least one element selected from the group consisting of zirconium, hafnium, columbium, vanadium, tantalum, molybdenum and manganese, but not to exceed 10% of tantalum, 3% of columbium and vanadium and 0.5% of molybdenum and manganese, balance substantially titanium, said alloy being characterized by high strength and ductility and by high thermal stability on aging exposure at 800-1000° F.

4. An alloy consisting essentially of about: 0.5 to 23% by weight of at least one alpha promoter selected from the group consisting of aluminum, tin and antimony, but not to exceed 7% of aluminum, and the maximum total content of the elements of said group being such that the percent of aluminum present plus  $\frac{1}{3}$  times the sum of the percents of tin and antimony present, shall not exceed 7%, said alloy also containing about 4 to 12% of zirconium, balance substantially titanium, said alloy being characterized by high strength and ductility and by good stability on prolonged aging exposure at about 800-1000° F.

5. An alloy consisting essentially of about: 0.5 to 23% by weight of at least one alpha promoter selected from the group consisting of aluminum, tin and antimony, but not to exceed 7% of aluminum, and the maximum total content of the elements of said group being such that the percent of aluminum present plus  $\frac{1}{3}$  times the sum of the percents of tin and antimony present, shall not exceed 7%, said alloy also containing about 4 to 12% of hafnium, balance substantially titanium, said alloy being characterized by high strength and ductility and by good stability on prolonged aging exposure at about 800-1000° F.

6. An alloy consisting essentially of about: 0.5 to 23% by weight of at least one alpha promoter selected from the group consisting of aluminum, tin, antimony, silver and indium, but not to exceed 7% of aluminum, 3% of indium, and 10% of silver, and the maximum total content of the alpha promoters of said group being such that the percent of aluminum present plus  $\frac{1}{3}$  times the sum of the percents of tin, antimony, silver and indium present, shall not exceed 7%, said alloy also containing about 0.1 to 10% of at least one beta promoter selected from the group consisting of tantalum, columbium, vanadium, molybdenum and manganese, but not to exceed 0.5% of molybdenum and manganese, balance substantially titanium, said alloy having a substantially all-alpha microstructure and being characterized by high strength and ductility and by good stability on prolonged aging at 800-1000° F.

7. An alloy consisting essentially of about: 0.5 to 23% by weight of at least one alpha promoter selected from the group consisting of aluminum, tin, antimony, silver and indium, but not to exceed 7% of aluminum, 10% of

silver and 3% of indium, and the maximum total content of the elements of said group present being such that the percent of aluminum present plus  $\frac{1}{3}$  times the sum of the percents of tin, antimony, silver and indium present, shall not exceed 7%, said alloy also containing up to 50% of metal of the group zirconium and hafnium, up to 10% tantalum, up to 3% columbium, up to 0.5% of metal of the group molybdenum and manganese, balance substantially titanium, said alloy having a substantially all-alpha microstructure, and being characterized by a tensile elongation of at least 10% on prolonged aging exposure at 800-1000° F.

8. An alloy consisting essentially of about: 0.5 to 23% by weight of at least one alpha promoter selected from the group consisting of aluminum, tin, antimony, silver and indium, but not to exceed 3% of indium, 7% of aluminum and 10% of silver, and the maximum content of elements of said group present being such that the percent of aluminum present plus  $\frac{1}{3}$  times the sum of the percents of tin, antimony, silver and indium present shall not exceed 7%, said alloy being characterized by a substantially all-alpha microstructure and by a tensile elongation of at least 10% on prolonged aging exposure at 800-1000° F.

9. An alloy consisting essentially of about: 3 to 6% aluminum, 4 to 12% zirconium, balance substantially titanium, characterized by high strength and ductility and high thermal stability on aging at about 800-1000° F.

10. An alloy consisting essentially of about: 3 to 6% aluminum, 4 to 10% tin, 5 to 12% zirconium and the balance substantially titanium, characterized by high strength and ductility and high thermal stability on aging at about 800-1000° F.

11. An alloy consisting essentially of about: 4 to 6% aluminum, 4 to 12% zirconium, 3 to 6% copper and the balance substantially titanium, characterized by high strength and ductility and high thermal stability on aging at about 800-1000° F.

12. An alloy consisting essentially of about: 0.5 to 23% by weight of at least one alpha promoter selected from the group consisting of aluminum, tin, antimony, silver and indium, but not to exceed 7% of aluminum, 3% of indium, 10% of silver, 20% of tin, and 18% of antimony, and the maximum total content of the elements of said group being such that the percent of aluminum plus  $\frac{1}{3}$  times the percents of tin, antimony, silver and indium present, shall not exceed 7%, said alloy also containing about 0.5 to 18% of at least one beta promoter, balance substantially titanium, said alloy being characterized by high strength, ductility and thermal stability and by good oxidation resistance at elevated temperatures up to 1800° F.

13. A titanium base alloy consisting essentially of about: 0.5 to 23% by weight of at least one alpha promoter selected from the group consisting of aluminum, tin, antimony, silver and indium, the total content of the elements of said group present being such that the percent of aluminum plus  $\frac{1}{3}$  the total percent of tin, antimony, silver and indium present is at least 7%, said alloy also containing 0.5 to 3% of metal of the group columbium and vanadium for improving stability of said alloy on aging at about 800 to 1000° F.

14. A titanium base alloy consisting essentially of about: 0.5 to 23% by weight of at least one alpha promoter selected from the group consisting of aluminum, tin, antimony, silver and indium, the total content of the elements of said group present being such that the percent of aluminum plus  $\frac{1}{3}$  the total percent of tin, antimony, silver and indium present is on the order of 6 to 10%, said alloy also containing 0.5 to 3% of metal of the group columbium and vanadium for improving stability of said alloy on aging at about 800-1000° F.

## References Cited in the file of this patent

## UNITED STATES PATENTS

|           |                     |               |
|-----------|---------------------|---------------|
| 2,596,486 | Jaffee et al. ----- | May 13, 1952  |
| 2,669,513 | Jaffee et al. ----- | Feb. 16, 1954 |
| 2,703,278 | Finlay -----        | Mar. 1, 1955  |
| 2,754,204 | Jaffee et al. ----- | July 10, 1956 |
| 2,754,205 | Jaffee et al. ----- | July 10, 1956 |
| 2,769,707 | Vordahl -----       | Nov. 6, 1956  |

## FOREIGN PATENTS

|                     |                |
|---------------------|----------------|
| France -----        | Feb. 24, 1954  |
| France -----        | Dec. 8, 1954   |
| France -----        | Dec. 8, 1954   |
| Great Britain ----- | Sept. 19, 1956 |

UNITED STATES PATENT OFFICE  
CERTIFICATE OF CORRECTION

Patent No. 2,892,705

June 30, 1959

Robert I. Jaffee et al.

It is hereby certified that error appears in the printed specification of the above numbered patent requiring correction and that the said Letters Patent should read as corrected below.

Column 1, line 39, for "Ti<sub>2</sub>Al" read -- Ti<sub>3</sub>(Al --; columns 3 and 4, TABLE I, under the heading "Test Temp., F.", sixth line from the bottom, for "76" read -- 75 --; columns 5 and 6, same TABLE I, continued, under the heading "Composition, Percent (Balance Titanium), third composition from the bottom, for the ingot number "1335" read -- 1435 --; same table, under the heading "Temp. F." line 7, for "700" read -- 800 --; same table, under the heading "Min. Creep Rate per hr.", second line from bottom, for "0.0060" read -- 0.0006 --; column 12, line 72, for "800-1000° C." read -- 800-1000° F. --.

Signed and sealed this 1st day of December 1959.

(SEAL)

Attest:

KARL H. AXLINE

Attesting Officer

ROBERT C. WATSON  
Commissioner of Patents